

## UNITED STATES PATENT OFFICE.

EDMOND JEAN EUGÉNE DUMOND, OF PARIS, FRANCE.

## PROCESS FOR PURIFYING, ENRICHING, OR REFINING CRUDE GRAPHITE.

No Drawing. Application filed April 8, 1925, Serial No. 21,701, and in France April 23, 1924.

Lumps or flakes of graphite are, as is well known, generally made up from a series of smaller flakes or fragments of pure graphite in aggregations united together by a silicious or aluminous cement. It follows that in order to purify or refine the mineral, it is necessary to employ a process for eliminating the largest possible proportion of the silicious or aluminous cement, whilst leaving the pure graphite in its original physical state, that is to say in the form of fine particles in which it existed when united in the coarser lumps submitted to treatment.

The present process has for its object the enrichment or refining of graphite by submitting the mineral to various treatments in succession, namely in the first place to a process of crushing then to trituration in a damp state in a tube mill or apparatus, then to separation in the damp state by sifting or passing through a sieve, and finally to flotation for the purpose of separating out the fine particles of refined graphite, those which are coarsest being again passed to the refining apparatus and again washed and sieved and floated in order to increase their richness or purity.

The trituration of the mineral, which has been previously crushed for instance to such a degree as to enable it to pass through a number 6 mesh, is effected in a tube mill or apparatus, the triturating means comprising metallic coned elements, sufficient water being injected at the time of treatment to render the mixture pasty. The object of this operation is to liberate or separate the constituent elements of the original lump or flake. The cementing material of the graphite particles is finely crushed, whilst the small fragments of graphite, by reason of their slimy nature remain almost unaffected.

Consequently, at the end of the treatment in the crushing apparatus, there is obtained a mixture consisting of pellicles of graphite, and silica, alumina and oxide of iron in a very finely pulverized condition, and these it is necessary to separate.

The sieving or sifting of the material is effected by means of a pneumatic vibrating sieve provided with a metallic net, of greater or less fineness, an atomizer or spray pro-

ducer being employed for constantly spraying with water the material under treatment, which increases to a considerable extent the efficacy of the sieving or sifting.

The two classes of material or products classified by the foregoing process are then passed to flotation chambers.

In this way graphite is obtained containing from 90 to 92% of carbon graphite of very high lubricating power. The graphite may be obtained of various degrees of coarseness, passing for example through 60, 120 or 200 mesh sieves.

The material which is coarser than 120 mesh is passed again through the crushing apparatus through the washer and through the flotation chambers, which gives a graphite of a greater purity than 95%.

If desired an even greater percentage of purity may be obtained by chemical treatment.

For this purpose the graphite obtained as above described is mixed with a determined proportion by weight of carbonate of soda according to the gangue content to be separated. The mixture is raised to 700° in a gas heated continuous kiln, and the operation may then be carried out in either of the two following methods:

(a) The product obtained from the kiln is passed again to the tube mill or apparatus and then may be sieved in the wet state and treated by flotation as explained above.

(b) If hydrochloric acid is obtainable at a commercial rate the material may be treated with a quantity of dilute acid sufficient for the soluble products, thus separating them together with silica in an extremely finely divided state. By washing, the soluble products and any excess of acid are removed, and the resulting material is sieved or sifted by means of the pneumatic vibrator to separate out the silica.

By these two processes graphite of a purity up to 99 or 99.5% is obtained.

I claim:

1. The art of refining graphite, comprising crushing the crude graphite, grinding the product wet, sifting the ground material while subjected to a spray of water, separating the graphite and chemically treating the sifted graphite for removal of residual gangue.

2. In the art of refining graphite, mixing partially refined graphite with sodium carbonate, heating the mixture to fusion and grinding the product wet.
3. In the art of refining graphite, mixing partially refined graphite with sodium carbonate, fusing the same, grinding the product, sifting it, treating it with dilute hydrochloric acid, washing it, sieving the resultant graphite wet, and finally separating the graphite by flotation.

In testimony that I claim the foregoing as my invention, I have signed my name.

EDMOND JEAN EUGÉNE DUMOND.